

# United States Patent

Oates

[15] 3,637,917

[45] Jan. 25, 1972

[54] **HERMETIC HIGH-CURRENT  
THERMINAL FOR ELECTRONIC  
DEVICES**

[72] Inventor: William Lee Oates, Bernardsville, N.J.

[73] Assignee: RCA Corporation

[22] Filed: Mar. 10, 1971

[21] Appl. No.: 122,672

[52] U.S. Cl.....174/152 GM, 174/50.61, 287/189.365

[51] Int. Cl.....H01b 17/26

[58] Field of Search.....174/50.56, 50.57, 50.58, 50.61,  
174/50.63, 152 GM; 29/472.9; 65/42, 59;  
287/189.365; 313/281, 332, 317, 318, 355; 339/144  
R, 144 T, 145 R, 145 D, 145 T

[56] References Cited

UNITED STATES PATENTS

1,265,665 5/1918 Jacoby.....287/189.365

|           |         |                   |               |
|-----------|---------|-------------------|---------------|
| 2,377,164 | 5/1945  | Lowit.....        | 174/50.61 UX  |
| 2,431,308 | 11/1947 | Cole.....         | 174/152 GM    |
| 2,446,277 | 8/1948  | Gordon.....       | 174/50.61 X   |
| 2,524,263 | 10/1950 | Kingston.....     | 174/50.61 X   |
| 2,885,826 | 5/1959  | Grieve et al..... | 174/152 GM UX |

FOREIGN PATENTS OR APPLICATIONS

912,115 5/1954 Germany.....174/152 GM

Primary Examiner—Laramie E. Askin  
Attorney—G. H. Bruestle

[57]

ABSTRACT

A metallic conductor extends through an insulating material disposed in an opening of a sleeve and has an expansion coefficient closely matching that of the insulating material. A relatively thick copper layer is disposed only on the outer end portions of the conductor.

6 Claims, 2 Drawing Figures



PATENTED JAN 25 1972

3,637,917



*Fig. 1*



*Fig. 2*

INVENTOR.  
**William L. Oates**  
BY  
*Herbert L. Allen*

ATTORNEY

## HERMETIC HIGH-CURRENT THERMAL FOR ELECTRONIC DEVICES

### BACKGROUND OF THE INVENTION

The present invention relates to electronic devices, and in particular, relates to high-current terminal means for such devices.

A wide variety of high-current terminals are presently used in the electronics industry. Many of these terminals are alike, however, in that a metallic conductor extends through an insulating material, as glass, which fills an opening in a sleeve, or package header. Because such terminals are generally required to operate at relatively high temperatures, the metals selected for the conductor generally have a thermal expansion coefficient closely matching that of the insulating material; to this end, Kovar and No. 52 alloy (52 percent nickel, balance iron) are frequently used.

However, these metals suffer relatively poor current-handling capabilities; thus, they are often combined with highly conductive metals which are otherwise thermally mismatched with the insulating material. In one example, the conductor has a small copper core with a thermally matched sheath surrounding the core. Yet another terminal employs a relatively large thermally matching core, with a thin copper sheet completely surrounding the thermally matched metal. But these and other terminals still suffer thermal matching and current handling capabilities.

Another terminal, not rated for high-current use, is employed in radiofrequency devices. This terminal has a conductor of a thermally matching metal extending through the insulating material. The outer portions of the conductor are plated with a very thin layer of a noble metal, such as gold or silver, in order to improve the skin conductivity of the terminal. However, such RF terminals are not capable of high-current operation as are other prior art terminals, such as those described above.

### SUMMARY OF THE INVENTION

The high-current terminal of the present invention comprises a sleeve member having two opposed surfaces with an opening between the surfaces, and with the opening filled with an insulating material. A metallic conductor extends through the insulating material and has end portions which extend away from each of the surfaces. The conductor has a coefficient of thermal expansion closely matching that of the insulating material. A relatively thick copper layer is disposed only on the end portions of the conductor.

### THE DRAWING

FIG. 1 is a cross-sectional view of the high-current terminal of the present invention.

FIG. 2 is a cross-sectional front view of the terminal of FIG. 1, taken along the lines 2-2.

### DETAILED DESCRIPTION

The high-current terminal of the present invention will be described with reference to FIGS. 1 and 2. The terminal, referred to generally as 10, includes a metal sleeve member 12 having opposed front and back surfaces 13 and 15, respectively, with an opening 14 between the two surfaces. The dimensions of the sleeve member 12 are not critical. By way of example, the sleeve member may be 0.10 inch thick between the two surfaces 13 and 15, and the opening 14 may be between 0.07 and 0.09 inch in diameter.

An insulating material 16 fills the opening 14. Preferably, the insulating material comprises a glass such as Corning Standard numbers 7052 or 9010, which glasses have thermal expansion coefficients of  $46 \times 10^{-7}$ /in./°C. and  $89 \times 10^{-7}$ /in./°C., respectively. A metallic conductor 18 extends through and is sealed to the insulating material. The conductor 18 has a thermal expansion coefficient which closely matches that of the insulating material 16. Preferably, the conductor comprises

Kovar or No. 52 alloy, which metals have thermal expansion coefficients of  $50 \times 10^{-7}$ /in./°C. and  $101 \times 10^{-7}$ /in./°C., respectively. The conductor may be between 20.0 and 30.0 mils in radius, for example.

5 The conductor 18 also includes end portions 20 and 22 which extend away from the two surfaces of the sleeve 13 and 15, respectively. The end portions 20 and 22 are coated with a relatively thick copper layer 24. Noting FIG. 2, the thermally matched conductor 18 defines a first radius  $r_1$ , and the outer periphery of the copper layer 24 defines a second radius  $r_2$ , which shares a common origin with the first radius  $r_1$ . In order that the terminal 10 can achieve an optimum current handling capability, it is preferable that radius  $r_2$  be at least 10.0 percent greater than radius  $r_1$ . Thus, if radius  $r_1$  is 20.0 mils, then radius  $r_2$  is at least 22 mils, and preferably about 25.0 mils. Since the thermally matched conductor 18 will not normally have a radius ( $r_1$ ) less than 20.0 mils, then the term "relatively thick" is intended to mean that the copper layer 24 is at least 2.0 mils thick, and preferably about 4.0 mils or thicker.

10 The sleeve member 12 may also have a relatively thick copper layer 26 deposited on the exposed surface thereof, which copper layer 26 is deposited on the sleeve member 12, during the preferred fabrication of the terminal 10, as described below. The terminal 10 is joined to an electronic device package header 28.

15 The metal conductor 18 may be sealed in the insulating material 16, and the insulating material may be disposed in the opening 14 of the sleeve 12, by fabrication techniques which are well known in the art. The relatively thick copper layer 24 may be deposited by any one of a variety of plating processes; for example, any electrolytic or electroless plating process. In addition, during the deposition of the copper layer 24, the copper layer 26 on the sleeve 12 is deposited to provide additional heat dissipation capability.

20 The terminal 10 of the present invention provides a good thermal expansion matching between the metal conductor 18 and the insulating material 16. In addition, the relatively thick copper layer which is disposed only on those portions 20 and 22 of the conductor 18 outside of the insulating material 16 provides a very high-current carrying capability; for example, a 5.0 mil copper layer on a 40.0 mil thermally matched conductor has about twice the current-handling capability of the 40.0 mil thermally matched conductor alone.

25 What is claimed is:

1. A high-current terminal comprising:  
a sleeve member having two opposed surfaces and an opening between said surfaces;  
an insulating material in said opening;  
a metallic conductor extending through said insulating material with end portions extending away from each said surface, said conductor having a coefficient of thermal expansion closely matching that of said insulating material; and  
30 a relatively thick copper layer disposed only on said end portions of said conductor.
2. A terminal according to claim 1 wherein said insulating material comprises glass.
3. A terminal according to claim 2 wherein said metallic conductor comprises an iron-nickel-cobalt alloy.
4. A terminal according to claim 2 wherein said metallic conductor comprises 52 percent nickel, balance iron.
5. A terminal according to claim 1 wherein said copper layer is at least 3.0 mils thick.
6. A high-current terminal comprising:  
a sleeve member having two opposed surfaces with an opening between said surfaces;  
an insulating material in said opening;  
a cylindrical metallic conductor having a first radius extending through said insulating material with end portions extending away from each said surface, said conductor having a coefficient of thermal expansion closely matching that of said insulating material;

a uniform copper layer disposed only on said end portions  
of said conductor, the outer periphery of said copper  
layer defining a second radius having a common origin  
with said first radius; and wherein  
said second radius is at least 10.0 percent greater than said 5  
first radius.

\* \* \* \* \*

10

15

20

25

30

35

40

45

50

55

60

65

70

75